

## UNITED STATES PATENT OFFICE

WILLIAM S. HEITMANN, OF PHILADELPHIA, PENNSYLVANIA

## PROCESS FOR MAKING TRACER COMPOSITIONS

No Drawing.

Application filed September 8, 1925. Serial No. 55,121.

(GRANTED UNDER THE ACT OF MARCH 3, 1883, AS AMENDED APRIL 30, 1928; 370 O. G. 757)

The invention described herein may be manufactured and used by or for the Government for governmental purposes without the payment to me of any royalty thereon.

5 The subject of this invention is a combustible and method of preparing the same.

The invention relates more particularly to combustibles for use in tracer projectiles, signals, illuminants and the like.

10 The main objects of the invention are to secure a more intimate admixture of the various elements going to make up the combustible mixture to secure a more uniform product that will load or mold easily, and to waterproof the resulting combustible.

In carrying out the invention, the components of the combustible mixture are mixed together, and the binder, which may be calcium resinate or any other metal salt of resinous acids or a resinous ester or other suitable binder which may be used either as a fuel, as a binder, as a waterproofing agent, or as any combination of these reasons, is dissolved in a suitable solvent, such as acetone or preferably

25 a non-inflammable solvent, such as carbon tetrachloride, and is then added in its dissolved condition to the mixed components of the combustible compound. After the ingredients are thus thoroughly mixed, the solvent is

30 driven off, preferably by evaporation, and the resultant mass is ground and sieved or otherwise thoroughly mixed so that there is formed a powder, the separate and individual grains of which are coated or impregnated, or both,

35 with the binder, which consequently is a more uniform burning mixture, one that is more easily loaded, and if a proper binder has been chosen, one which is almost completely non-hygroscopic. In loading or using such a re-

40 sultant powder it is supposed that it will be forced by pressure into a container or will be molded by pressure into pellets or other shapes. By the use of this invention greater

45 ease will be secured in measuring this material, in pressing it as outlined above, and the resulting shapes or loaded containers will be waterproof. By the use of a proper binder, a pellet can be secured which has a hardness

50 several times greater than that of lead, and which will have sufficient tensile strength that

it will not shatter with the shock of an explosion from a propelling charge when fired from a gun or rocket tube.

I claim:

1. The method of preparing a tracer mixture embodying mixing combustible ingredients, dissolving a metallic resinate in a solvent, adding the solution thus obtained to the mixed ingredients and incorporating the same, driving off the solvent, grinding the resultant mass, grading the resultant powder, then pressing the same to the desired form. 55

2. The method of preparing a tracer mixture embodying mixing the combustible ingredients, dissolving a binder consisting of a metallic resinate in a solvent, adding the solution thus obtained to the mixed ingredients and incorporating the same, driving off the solvent, grinding and grading the resultant mass, then pressing the same to the desired form. 60 65

3. A method of preparing a tracer mixture embodying mixing the combustible ingredients, dissolving a metallic resinate in a solvent, adding the solution to the ingredients and incorporating the same, driving off the solvent then grinding and grading the resultant mass. 70 75

WILLIAM S. HEITMANN. 80

55

60

65

70

75

80

85

90

95

100